

Patented June 13, 1939

2,162,495

# UNITED STATES PATENT OFFICE

2,162,495

## CONCENTRATION OF ORES

William Trotter, San Francisco, and Eltoft Wray Wilkinson, Berkeley, Calif., assignors to Minerals Separation North American Corporation, New York, N. Y., a corporation of Maryland

No Drawing. Original application August 20, 1934, Serial No. 740,600. Divided and this application January 24, 1938, Serial No. 186,586

17 Claims. (Cl. 209—166)

This application is a division of our co-pending application Serial No. 740,600, filed August 20, 1934.

The present invention relates to a novel process of ore concentration and is herein illustrated as applied to the concentration of both metalliferous and so-called non-metallic ores.

The process of the present invention has proved especially useful in concentrating phosphate-bearing ores.

In accordance with the invention, ores are concentrated by procedures involving their admixture with a non-frothing organic liquid immiscible with water, such as fuel oil, and a thiocarbonic acid derivative containing the residue of an aliphatic alcohol of at least twelve carbon atoms. Such organic-substituted compounds may, for example, be alkali metal and alkaline earth metal xanthates of the stated number of carbon atoms in the hydrocarbon radical contained therein. The aliphatic alcohols capable of use in producing the organic-substituted compounds of the present invention may be normal primary alcohols, but other types of alcohols may also be used. The organic-substituted or hydrogen-replacing groups in these compounds thus not only comprise simple alkyl radicals, but may also consist of the residues of unsaturated olefinic alcohols. Examples of organic-substituted compounds which may be used in the process of the present invention are alkali metal and alkaline earth metal salts of xanthic acids containing the alcohol radicals lauryl, cetyl, myristyl, oleyl, etc.

Instead of thiocarbonic acid derivatives, it has also been found possible to employ with non-frothing water-immiscible organic liquids derivatives of phosphoric acid similarly containing aliphatic alcohol residues of at least twelve carbon atoms, e. g., the acid esters of phosphoric acid with such alcohols as lauryl, cetyl, myristyl, and oleyl alcohols, as well as the alkali metal and alkaline earth metal salts of such acid esters. However, the claims of this application do not cover the use with non-frothing water-immiscible organic liquids of these phosphoric acid derivatives, which are separately claimed in our aforementioned application Ser. No. 740,600.

Many non-frothing organic liquids, substantially insoluble in or immiscible with water in the proportions used, may be employed to carry out the process of the present invention by cooperating with the organic-substituted compounds herein described. Such liquids contain no substantial amounts of free fatty acids. Such widely varying types of non-frothing substantially water-immiscible organic liquids as fuel oil, kerosene, dipentene (a terpene hydrocarbon), crude solvent naphtha (from coal tar), water gas tar, and carbon tetrachloride have proved useful in carrying out the process of the present invention.

Fuel oil, however, on account of its low cost, is generally preferred.

The organic-substituted compounds used in the process of the present invention have certain characteristics of soap and are in general capable of operating as frothing agents. However, the principal function of the organic-substituted compounds used in the process of the present invention is to make the non-frothing water-immiscible organic liquids also used effective by causing those liquids to adhere selectively to the mineral values in the ore.

The use of xanthates and other thiocarbonic acid derivatives in the flotation concentration of sulphide and other metallic minerals is well known in the art. And we are well aware of the fact that in these prior processes the efficiency of such compounds becomes less as the number of carbon atoms included in the alcohol employed in their preparation increases to more than about seven. On the other hand, it has been found that, in order to be useful in the process of the present invention, xanthates and other thiocarbonic acid derivatives must have twelve or more carbon atoms in their alcoholic radical. The "lower" organic-substituted thio-carbonic acid compounds which are best in the flotation concentration of sulphides and other metallic minerals are of no value whatever in the process of the present invention.

The organic-substituted compounds used in the process of the present invention need not be pure compounds. For instance, the alcohols used in making them may be of commercial grades containing substantial amounts of other alcohols, which results in the production of mixtures of organic-substituted compounds of varying carbon content in the substituted radical. The process of the present invention may obviously be carried out with such mixtures, provided the organic-substituted compounds having radicals of at least twelve carbon atoms largely predominate.

It is also to be understood that the process of the present invention is not limited to the exclusive use of the organic-substituted compounds herein described with their cooperating non-frothing water-immiscible liquids organic. Other agents known to those skilled in the art may be employed to contribute their own peculiar properties, such as frothing ability, pH control, etc., whereby the best conditions for the exercise of the intended functions of the organic-substituted compounds herein described and their cooperating non-frothing water-immiscible organic liquids may be obtained.

In carrying out the process of the present invention, addition to the ore of the various reagents used may be made with the ore either in a state of dryness or in the form of an aqueous pulp. In either case, of course, the subsequent

step of separating the mineral values is carried out in an aqueous pulp of the ore. For this separation various physical forms of concentration have been found useful, which include froth flotation, tabling, and hydraulic classification.

In preparing the ore for treatment by the process of the invention, it is in general desirable that it be largely deslimed, its desliming greatly minimizing the consumption of the agents used, improving the results obtained, and rendering the process commercially practicable. In most cases, the crude ore is first subjected to a preliminary grinding operation, after which slimes are removed.

Examples will now be given describing certain tests which have been made in carrying the invention into effect, it being understood that the reagent proportions indicated in each example are expressed in the usual manner as pounds per ton (2000 lbs.) of dry material treated.

*Example 1.*—Valley Forge Cement Company classifier overflow, consisting mainly of finely crushed limestone and silica, was mixed with 2.2 lbs. per ton of potassium cetyl xanthate dissolved in water, the quantity of water being such as to produce a pulp of 45% solids. To this pulp were then added 13 lbs. per ton of fuel oil. After thorough mixing, the pulp was thinned and frothed in a laboratory-size subaeration flotation machine, another 2.2 lbs. per ton of potassium cetyl xanthate being added after about one minute of froth removal, the total period of which was about two minutes. The heads contained 74.1%  $\text{CaCO}_3$  and 20.26% insoluble matter. The concentrates carried 55.0% of the total calcite content of the heads in a product containing 85.5%  $\text{CaCO}_3$  and 8.2% insolubles.

In each of the following six examples, Florida phosphate ore, screened to pass 20-mesh and deslimed, was first mixed dry with fuel oil and thereafter mixed dry or in a thick pulp with an alkali metal xanthate. The mixture was then diluted and the B. P. L. values (tricalcium phosphate) removed therefrom by flotation. The material floated in these tests was either of the nature of a froth or of the nature of a heavy flocculated float.

*Example 2.*—For the purpose of this test, potassium cetyl xanthate was used to cooperate with the fuel oil, the above-mentioned phosphate ore being treated with these agents in the amounts of 1.5 lbs. per ton of the xanthate and 11.2 lbs. per ton of the fuel oil. From heads containing 27.8% B. P. L., concentrates assaying 77.0% B. P. L. and tailings 10.2% were obtained, representing a B. P. L. recovery of 72.9%.

*Example 3.*—In this test, using 2 lbs. per ton of potassium myristyl xanthate and 11.2 lbs. per ton of fuel oil, the concentrates assayed 73.6% B. P. L. and the tailings 6.6%. The heads contained 27.3% B. P. L., the recovery being 83.3%.

*Example 4.*—When 1.5 lbs. per ton of potassium myristyl xanthate and 9.4 lbs. per ton of fuel oil were used instead of the larger amounts, the B. P. L. assay of the concentrates was 75.8% and that of the tailings 9.6%. The B. P. L. recovery was 74.1%, the content of the heads being 27.2%.

*Example 5.*—In this instance, using 2 lbs. of potassium lauryl xanthate and 24.4 lbs. of fuel oil, both per ton, concentrates assaying 74.0% B. P. L. and tailing 11.0% were obtained from heads of 26.5%, the recovery being 68.7%.

*Example 6.*—With the amount of potassium lauryl xanthate increased to 2.5 lbs. per ton and

that of fuel oil decreased to 20.5 lbs. per ton, the concentrates assayed 74.0% B. P. L. and the tailings 7.8%, representing a B. P. L. recovery of 79.6%, the content of the heads being 27.1%.

*Example 7.*—For this test, 1.5 lbs. of potassium oleyl xanthate and 11.2 lbs. of fuel oil, both per ton, were employed. The heads contained 26.4% B. P. L., the concentrates 74.4%, and the tailings 5.2%, representing a B. P. L. recovery of 86.4%.

*Example 8.*—Another lot of the same deslimed phosphate ore was oiled dry with 11.2 lbs. per ton of fuel oil and 2 lbs. per ton of potassium myristyl xanthate, wetted to a thick pulp, mixed with more water to form a freely flowing pulp, and subjected to concentration on a Wilfley table, the phosphate values coming off the side of the table and the tailings coming off the end. The concentrates came off partly as a surface film and partly as floccules mostly suspended below the surface of the water. They were mixed with a further addition of 0.5 lb. of potassium myristyl xanthate and 1.7 lbs. of fuel oil, both per ton, and subjected to further treatment on the table to yield a finished product of concentration. By this last operation, a middlings product was also obtained, which came off the end of partly at the table and partly at the extreme end of the lower side. The results are shown in the following table, in which the high recovery will be noted:

|            | Percent weight | Percent assay B. P. L. | Percent recovery B. P. L. | 35 |
|------------|----------------|------------------------|---------------------------|----|
| Heads..... | 100.00         | 27.7                   | 100.0                     |    |
| Concs..... | 38.65          | 64.0                   | 89.3                      |    |
| Midds..... | 7.55           | 30.6                   | 8.4                       |    |
| Tails..... | 53.80          | 1.2                    | 2.3                       |    |

*Example 9.*—In this test, a xanthate containing an alkyl group with twelve carbon atoms proved useful on the highly refractory oxidized lead-silver ore of Naica mines of Mexico. This ore, ground to pass 48-mesh and then deslimed, was added to a little more than its own weight of water containing 3 lbs. of potassium lauryl xanthate per ton of ore. Thereafter, there were added 14.9 lbs. per ton of fuel oil, stirring being carried out for one-quarter minute. The resulting mixture was then diluted and concentrates removed by flotation. Another 3 lbs. per ton of potassium lauryl xanthate was added to the remaining pulp, admixture carried out, and further concentrates removed by flotation. These were added to the first concentrates, the combined concentrates being then subjected to flotation so as to separate a final product of concentration therefrom. A middlings product was also obtained by this last operation, which was carried out without adding further agents. The results of the test were as follows:

|            | Percent weight | Assays     |            | Distribution |            | 65 |
|------------|----------------|------------|------------|--------------|------------|----|
|            |                | Ag oz./ton | Pb percent | Ag percent   | Pb percent |    |
| Heads..... | 100.0          | 17.27      | 11.59      | 100.0        | 100.0      |    |
| Concs..... | 14.0           | 80.00      | 43.00      | 64.8         | 52.0       | 70 |
| Midds..... | 18.0           | 13.76      | 16.60      | 14.4         | 25.8       |    |
| Tails..... | 68.0           | 5.28       | 3.90       | 20.8         | 22.2       |    |

*Example 10.*—Another lot of the same ore, also of 48-mesh and nearly deslimed, was added to a

little more than its own weight of water containing potassium oleyl xanthate at the rate of 3 lbs. per ton of the ore. The mixture was then stirred in a flotation machine for one-fourth 5 minute with an added 14.9 lbs. of fuel oil per ton of the ore, diluted, and agitated for a removal of "1st concentrates." Two pounds more, per ton, of the same xanthate were added to the remaining pulp, admixture carried out, and 10 "2nd concentrates" removed. In this test, the heavily oiled floating material was held up partly as a bubble-supported mat and partly as a froth. The results of the test are shown in the following table:

|                | Percent weight | Assays     |            | Distribution |            |
|----------------|----------------|------------|------------|--------------|------------|
|                |                | Ag oz./ton | Pb percent | Ag percent   | Pb percent |
| Heads.....     | 100.0          | 17.77      | 12.04      | 100.00       | 100.0      |
| 1st concs..... | 10.1           | 95.88      | 32.80      | 54.50        | 27.5       |
| 2nd concs..... | 10.7           | 31.15      | 42.40      | 18.75        | 37.7       |
| Tails.....     | 79.2           | 6.00       | 5.30       | 26.75        | 34.8       |

25 *Example 11.*—Evans Wallower zinc blende ore, ground to pass 48-mesh and then deslimed, was first mixed dry with 11.2 lbs. per ton of fuel oil and thereafter added to a little more than its own weight of water containing 2 lbs. of potassium cetyl xanthate per ton of ore. The mixture was thoroughly stirred, after which it was diluted and subjected to flotation, a heavily flocculated mat-like float being removed. Without further agents, this float was retreated to 30 yield a finished product of concentration and a middlings product. The following results were obtained:

|            | Percent weight | Percent Zn assay | Percent Zn recovery |    |    |
|------------|----------------|------------------|---------------------|----|----|
|            |                |                  |                     | 40 | 45 |
| Heads..... | 100.0          | 5.53             | 100.0               |    |    |
| Concs..... | 7.8            | 55.20            | 77.9                |    |    |
| Midds..... | 4.3            | 10.00            | 7.8                 |    |    |
| Tails..... | 87.9           | 0.90             | 14.3                |    |    |

50 *Example 12.*—When potassium myristyl xanthate was substituted for the cetyl xanthate of Example 11, the concentrates carried 55.0% zinc and the tailings 0.5%.

55 In each of the following three examples a water-immiscible liquid other than fuel oil was employed.

60 *Example 13.*—Florida phosphate ore, ground to pass 35-mesh and deslimed, was added to its own weight of water with 2.5 lbs. of potassium lauryl xanthate and 10.9 lbs. of xylol, both per ton of ore. This mixture was stirred for fifteen seconds, whereafter it was diluted and subjected to flotation, a well flocculated froth high in phosphate being removed. The results of the test are indicated in the following table:

|            | Percent weight | Percent assay B. P. L. | Percent recovery B. P. L. |    |    |
|------------|----------------|------------------------|---------------------------|----|----|
|            |                |                        |                           | 65 | 70 |
| Heads..... | 100.0          | 26.9                   | 100.0                     |    |    |
| Concs..... | 31.6           | 77.2                   | 90.6                      |    |    |
| Tails..... | 68.4           | 3.7                    | 9.4                       |    |    |

75 *Example 14.*—When 29.6 lbs. per ton of carbon tetrachloride were used in place of the xylol of Example 13, all other factors being the same, a flocculent froth of the phosphate values was again produced, though the results might have

been better by varying the reagent amounts, these results being as follows:

|            | Percent weight | Percent assay B. P. L. | Percent recovery B. P. L. | 5  |
|------------|----------------|------------------------|---------------------------|----|
| Heads..... | 100.0          | 25.3                   | 100.0                     |    |
| Concs..... | 22.2           | 72.1                   | 63.4                      |    |
| Tails..... | 77.8           | 11.9                   | 36.6                      | 10 |

10 *Example 15.*—Here 10.8 lbs. per ton of pure turpentine were used instead of the xylol of Example 13. The conditions of the test were otherwise the same, a flocculated froth of phosphate being readily obtained with the following results:

|            | Percent weight | Percent assay B. P. L. | Percent recovery B. P. L. | 15 |
|------------|----------------|------------------------|---------------------------|----|
| Heads..... | 100.0          | 23.77                  | 100.0                     |    |
| Concs..... | 32.5           | 64.70                  | 88.3                      |    |
| Tails..... | 67.5           | 4.10                   | 11.7                      | 20 |

25 Retreatment of the concentrates obtained in the last three examples would have raised their grade without materially increasing the loss in phosphate values.

30 While the foregoing examples describe tests carried out with potassium compounds of xanthic acids, the sodium, barium compounds are equally as effective in the process of the present invention. The barium and ammonium compounds are also useful in the process of the present invention, although the sodium and potassium compounds are preferred.

35 Having thus described certain embodiments of the invention, what is claimed is:

1. The process of concentrating ores which comprises admixing with the ore, in a suitably divided state and relatively free from slimes, a non-frothing organic liquid immiscible with water and a derivative of a thiocarbonic acid containing the residue of an aliphatic alcohol of at 40 least twelve carbon atoms; and separating in an aqueous pulp the mineral values from the ore.

2. The process of concentrating ores which comprises admixing with the ore, in a suitably divided state and relatively free from slimes, a non-frothing organic liquid immiscible with water and a derivative of a thiocarbonic acid containing an organic radical of the class consisting of saturated and unsaturated straight-chain alkyl groups of at least twelve carbon atoms; and separating in an aqueous pulp the mineral values from the ore. 50

3. The process of concentrating ores which comprises admixing with the ore, in a suitably divided state and relatively free from slimes, a non-frothing organic liquid immiscible with water and a compound included in the class consisting of the alkali-metal and alkaline-earth-metal salts of acids derived from thiocarbonic acids by replacing one of their hydrogen atoms with the residue of an aliphatic alcohol of at 60 least twelve carbon atoms; and separating in an aqueous pulp the mineral values from the ore.

4. The process of concentrating ores which comprises admixing with the ore, in a suitably divided state and relatively free from slimes, a non-frothing organic liquid immiscible with water and a compound included in the class consisting of the alkali-metal and alkaline-earth-metal salts of dithio-carbonic acids having one of their hydrogen atoms replaced by the residue of 70 75

an aliphatic alcohol of at least twelve carbon atoms; and separating in an aqueous pulp the mineral values from the ore.

5. The process of concentrating ores which comprises admixing with the ore, in a suitably divided state and relatively free from slimes, a non-frothing organic liquid immiscible with water and a compound included in the class consisting of alkali-metal and alkaline-earth-metal xanthates containing as their hydrocarbon radicals the residues of saturated and unsaturated alcohols of at least twelve carbon atoms; and separating in an aqueous pulp the mineral values from the ore.

15. 6. The process of concentrating ores which comprises admixing with the ore, in a suitably divided state and relatively free from slimes, a non-frothing organic liquid immiscible with water and an alkali-metal xanthate containing as the hydrocarbon radical therein a straight-chain alkyl group of at least twelve carbon atoms; and separating in an aqueous pulp the mineral values from the ore.

7. The process of concentrating ores which 25 comprises admixing with the ore, in a suitably divided state and relatively free from slimes, a non-frothing organic liquid immiscible with water and a compound included in the class consisting of alkali-metal and alkaline-earth-metal xanthates containing as their hydrocarbon radicals the residues of saturated and unsaturated alcohols of at least twelve carbon atoms; and subjecting the ore in the form of an aqueous pulp to froth flotation so as to remove the mineral 35 values therefrom.

8. The process of concentrating non-metallic ores which comprises admixing with the non-metallic ore, in a suitably divided state and relatively free from slimes, a non-frothing organic liquid immiscible with water and an alkali-metal xanthate containing as the hydrocarbon radical therein a straight-chain alkyl group of at least twelve carbon atoms; and separating in an aqueous pulp the non-metallic mineral values from the ore.

45. 9. The process of concentrating phosphate-bearing ores which comprises admixing with the phosphate-bearing ore, in a suitably divided state and relatively free from slimes, a non-frothing organic liquid immiscible with water and an alkali-metal xanthate containing as the hydrocarbon radical therein a straight-chain alkyl group of at least twelve carbon atoms; and separating in an aqueous pulp the phosphate values 55 from the ore.

10. The process of concentrating ores which comprises admixing with the ore, in a suitably divided state and relatively free from slimes, a non-frothing organic liquid immiscible with water and an alkali-metal salt of a xanthic acid containing as the hydrocarbon radical therein the residue of an unsaturated olefinic alcohol of at least twelve carbon atoms. and separating in an aqueous pulp the mineral values from the ore.

65. 11. The process of concentrating non-metallic ores which comprises admixing with the non-

metallic ore, in a suitably divided state and relatively free from slimes, a non-frothing organic liquid immiscible with water and an alkali-metal salt of a xanthic acid containing as the hydrocarbon radical therein the residue of an unsaturated olefinic alcohol of at least twelve carbon atoms; and separating in an aqueous pulp the non-metallic mineral values from the ore.

5. 12. The process of concentrating ores which comprises admixing a thick aqueous pulp, relatively free from slimes, of suitably divided particles of the ore with a non-frothing water-immiscible organic liquid and an alkali-metal xanthate containing as the hydrocarbon radical therein a straight-chain alkyl group of at least twelve carbon atoms; and separating the mineral values from the pulp.

10. 13. The process of concentrating non-metallic ores which comprises admixing a thick aqueous pulp, relatively free from slimes, of suitably divided particles of the non-metallic ore with a non-frothing water-immiscible organic liquid and an alkali-metal xanthate containing as the hydrocarbon radical therein a straight-chain alkyl group of at least twelve carbon atoms; and separating the non-metallic mineral values from the pulp.

15. 14. The process of concentrating ores which comprises admixing with the ore, in a suitably divided state and relatively free from slimes, a non-frothing organic liquid immiscible with water and a compound of the following general formula:

RO.C.SM  
S

35

wherein R represents the residue of a straight-chain aliphatic alcohol of at least twelve carbon atoms and M represents hydrogen or an alkali metal or an alkaline earth metal; and separating in an aqueous pulp the mineral values from the ore.

40. 15. The process of concentrating ores which comprises admixing with the ore, in a suitably divided state and nearly free from slimes, a non-frothing organic liquid immiscible with water and an alkali-metal oleyl xanthate; and separating in an aqueous pulp the mineral values from the ore.

45. 16. The process of concentrating ores which comprises admixing with the ore, in a suitably divided state and relatively free from slimes, a non-frothing organic liquid immiscible with water and an alkali-metal lauryl xanthate; and separating in an aqueous pulp the mineral values from the ore.

55. 17. The process of concentrating ores which comprises admixing with the ore, in a suitably divided state and relatively free from slimes, a non-frothing organic liquid immiscible with water and an alkali-metal cetyl xanthate; and separating in an aqueous pulp the mineral values from the ore.

60. WILLIAM TROTTER.  
ELTOFT WRAY WILKINSON. 65

CERTIFICATE OF CORRECTION.

Patent No. 2,162,495.

June 13, 1939.

WILLIAM TROTTER, ET AL.

It is hereby certified that error appears in the printed specification of the above numbered patent requiring correction as follows: Page 1, first column, line 7, for "and and" read and; same page, second column, line 47, for the words "liquids organic" read organic liquids; page 2, second column, lines 27 and 28, for the words "the end of partly at" read partly at the end of; page 3, second column, line 31, strike out the comma and word ", barium"; and that the said Letters Patent should be read with this correction therein that the same may conform to the record of the case in the Patent Office.

Signed and sealed this 1st day of August, A. D. 1939.

(Seal)

Henry Van Arsdale,  
Acting Commissioner of Patents.